

## UNITED STATES PATENT OFFICE

2,192,118

## ACID DIAMINO-TRIPHENYL-METHANE DYE-STUFFS

Paul Herbert Wolff, deceased, late of Frankfort-on-the-Main-Hochst, Germany, by Richard Wenzel, administrator, Frankfort-on-the-Main-Hochst, Germany, and Hans Moehrke and Gustav Schäfer, Frankfort-on-the-Main-Hochst, Germany, assignors to General Aniline & Film Corporation, a corporation of Delaware

No Drawing. Application March 21, 1939, Serial No. 263,182. In Germany March 23, 1938

5 Claims. (Cl. 260—394)

The present invention relates to acid diamino-triphenyl-methane dyestuffs.

We have found that valuable acid diamino-triphenyl-methane dyestuffs may be obtained by using, in processes known per se, aromatic amines containing, at the nitrogen, aliphatic radicals having 8 to 18 carbon atoms which may be branched or straight alkyl groups. There are obtained, for instance, dyestuffs of the following 10 general formula:



20 wherein  $n$  means one of the numbers one and two, wherein  $X_1$  represents an alkyl group containing 8 to 18 carbon atoms,  $X_2$  represents a member of the group consisting of hydrogen, alkyl and aralkyl of the benzene series,  $X_3$  represents a member of the group consisting of aryl of the benzene series and alkyl containing 8 to 18 carbon atoms and 30  $Y$  represents a member of the group consisting of hydrogen and alkyl.

Compared with known dyestuffs (cf. "Farbstofftabellen", Schultz, 7th ed., Nos. 769, 770 and 771) containing at the nitrogen, alkyl groups with 1 to 4 carbon atoms, the new acid dyestuffs are 35 distinguished by better tinctorial properties, for instance fastness to water, to washing, to seawater and to transpiration.

As known processes for the preparation of acid 40 triphenyl-methane dyestuffs, the following are mentioned:

(1) Melting ketones with primary, secondary or tertiary amines, whereby each of the components may contain one or more sulfo-groups 45 and/or the dyestuff may be subjected to a subsequent sulfonation.

(2) Condensing benzhydrols or benzhydrole-sulfonic acids (obtainable, for instance, from tetramethyl-diamino-diphenyl-methane or from 50 diethyl-dibenzyl-diamino-diphenyl-methane-disulfonic acid by oxidation to the hydrole) with substituted aromatic, isocyclic or heterocyclic bodies, for instance amines, phenols or sulfonic acids and oxidizing the leuco compounds obtained so as to form the dyestuff.

(3) Condensing aldehydes of the benzene or naphthalene series with primary, secondary or tertiary amines, whereby acid groups may be present in the components or may subsequently be introduced into the leuco compounds obtained and oxidizing the leuco compounds so as to form the dyestuff.

The following examples serve to illustrate the invention, but they are not intended to limit it thereto; the parts are by weight:

(1) 16 parts of alpha-naphthaldehyde and 86.2 parts of dodecylbenzyl-aniline-sulfonic acid of the formula:



20 (obtainable from dodecylaniline by reaction with benzyl-chloride and sulfonation at ordinary temperature with six times its weight of fuming sulfuric acid containing 5% of sulfuric anhydride) are heated at 100° C. for 60 hours with 120 parts of water and 5.5 parts of anhydrous sodium carbonate. The leuco dyestuff formed is precipitated with acid, dissolved in about 600 parts of water and the calculated amount of caustic soda solution and oxidized with lead dioxide in N-sulfuric acid so as to obtain the 30 dyestuff. It yields a very clear green tint and is distinguished by a good levelling power.

25 (2) A mixture of 72.2 parts of dodecyl-benzaniline, 26.6 parts of benzaldehyde-2,4-disulfonic acid and 525 parts of sulfuric acid of 60% strength is heated at 100° C.—105° C. for 80 hours. The leuco-sulfonic acid thus obtained is filtered with suction and transformed into its sodium salt by dissolving it in caustic soda solution. By 35 addition of 50 parts of oxalic acid, 90 parts of glacial acetic acid and 14.5 parts of sodium bichromate to the solution at a temperature of 50° C.—100° C., a dyestuff is formed which may easily be isolated by salting out. It dyes wool green-blue tints and is distinguished by a very good 45 levelling power.

(3) 26.6 parts of benzaldehyde-2,4-disulfonic acid and 47 parts of ethyl-octyl-aniline of the following formula:



55 are condensed in 250 parts of sulfuric acid of

10% strength at 100° C. for about 100 hours. The leuco acid thus obtained is oxidized with sodium bichromate at 90° C.-100° C., in the presence of sulfuric acid and oxalic acid, so as to obtain the dyestuff. By salting out, it separates in the form of its sodium salt; after drying, the dyestuff constitutes a blue powder which dyes wool and silk, in an acid bath, blue tints which are distinguished by a good fastness to washing, fulling and sea-water. The dyestuff has the following probable formula:



Similar dyestuffs are obtained by using ethyl-dodecyl-aniline or butyl-dodecyl-aniline instead of ethyl-octyl-aniline.

25 (4) 26.6 parts of benzaldehyde-2,4-disulfonic acid and 59 parts of octyl-benzyl-aniline are condensed in 250 parts of sulfuric acid of 10% strength at 100° C. for about 100 hours, and the reaction mixture is worked up as indicated in Example 3.

30 The dyestuff thus obtained dyes wool blue tints which are distinguished by a very good fastness to sea-water. It probably corresponds with the following formula:



45 (5) 26.6 parts of benzaldehyde-2,4-disulfonic acid and 44 parts of mono-octyl-ortho-toluidine are condensed in 250 parts of sulfuric acid of 10% strength at a temperature of 100° C. for about 120 hours. The leuco acid is separated and then oxidized, in known manner, by means of manganese dioxide, in the presence of dilute sulfuric acid. The dyestuff separates in the form of the sodium salt. It dyes wool, in an acid bath, reddish-blue tints which are distinguished by a good fastness to washing, fulling and sea-water.

50 The dyestuff corresponds with the following probable formula:



65 If, instead of octyl-ortho-toluidine, there are used 55 parts of dodecyl-ortho-toluidine or 72 parts of octadecyl-ortho-toluidine, dyestuffs having similar properties of fastness are obtained.

70 (6) 16.8 parts of benzaldehyde-ortho-sulfonic acid and 86.2 parts of dodecyl-benzyl-aniline-sulfonic acid are condensed in 200 parts of water at 90° C.-100° C. for about 100 hours. The leuco acid is filtered with suction and oxidized with 75 sodium bichromate in dilute acetic acid in the

presence of oxalic acid so as to form the dyestuff. After salting out, the dyestuff is obtained in the form of its sodium salt; it dyes wool, in an acid bath, blue-green tints having a good fastness, to wet processing.

5 If octyl-benzyl-m-toluidine-sulfonic acid or dodecyl-benzyl-m-toluidine-sulfonic acid are used instead of dodecyl-benzyl-aniline-sulfonic acid, there are obtained dyestuffs having similar properties of fastness.

10 (7) A mixture of 35 parts of 4-chlorobenzophenone-chloride 2'-sulfonic acid, 23.3 parts of ethyl-octyl-aniline, 150 parts of benzene and 16 parts of zinc chloride is heated for 20 hours on the water-bath, while stirring under reflux. The 15 condensation product separates in the form of a dark red resin. It is washed with benzene and dried.

15 49 parts of the condensation product thus obtained are heated at 100° C.-105° C., for about 20 4½ hours, together with 200 parts of para-phenetidine. The green dyestuff is isolated by stirring the whole several times with hydrochloric acid; it is then washed with water until neutral and dried.

20 The dyestuff obtained in the form of the mono-sulfonic acid is dissolved in five times its weight of concentrated sulfuric acid and transformed into a disulfonic acid by heating the solution for 2-3 hours at 40° C. When precipitated in the usual manner, the dyestuff constitutes a green 25 powder it dyes wool, in an acid bath, clear green tints which are distinguished by a good fastness to wet processing.

25 We claim:

30 1. The compounds of the general formula:



45 wherein n means one of the numbers one and two,

wherein X1 represents an alkyl group containing 8 to 18 carbon atoms,

X2 represents a member of the group consisting of hydrogen, alkyl and aralkyl of the benzene 50 series, X3 represents a member of the group consisting of aryl of the benzene series and alkyl containing 8 to 18 carbon atoms and

Y represents a member of the group consisting of hydrogen and alkyl.

55 2. The compounds of the general formula:



65 wherein X1 represents an alkyl group containing 8 to 18 carbon atoms,

X2 represents a member of the group consisting of hydrogen, alkyl and aralkyl of the benzene 70 series,

X3 represents a member of the group consisting of aryl of the benzene series and alkyl containing 8 to 18 carbon atoms and

Y represents a member of the group consisting of hydrogen and alkyl.

5

10

25

30

35

40

45

50

55

60

65

70

75

## 3. The compound of the formula:



being a blue powder which dyes wool and silk, in an acid bath, blue tints which are distinguished by a good fastness to washing, fulling and to sea-water.

## 15. 4. The compound of the formula:



being a dyestuff which dyes wool blue tints which are distinguished by a very good fastness to sea-water.

## 5. The compound of the formula:



being a dyestuff which dyes wool, in an acid bath, reddish-blue tints which are distinguished by a good fastness to washing, fulling and sea-water.

RICHARD WENZEL,  
As administrator of Paul Herbert Wolf, Deceased.

HANS MOEHRKE.

GUSTAV SCHÄFER. 25